

May 25, 1926.

1,585,716

P. L. HULIN

## PREPARATION OF SODIUM

Filed Nov. 26, 1923

3 Sheets-Sheet 1

Fig. 1. Fig. 2. Fig. 3.



Fig. 4.  A diagram showing a large rectangle divided into four quadrants by a horizontal and a vertical line. The center square where the lines intersect is shaded black.



၁၅



Fig. 4.



*INVENTOR*

PAUL LÉON HULIN

BY

*Lotta, Kehlenbeck & Matthe*  
ATTORNEYS

**ATTORNEYS**

May 25, 1926.

1,585,716

P. L. HULIN

PREPARATION OF SODIUM

Filed Nov. 26, 1923

3 Sheets-Sheet 2

Fig. 7.



Fig. 8.



Fig. 9.



INVENTOR  
PAUL LÉON HULIN  
BY  
*Loftus, Schubert & Motte*  
ATTORNEYS

May 25, 1926.

1,585,716

P. L. HULIN

PREPARATION OF SODIUM

Filed Nov. 26, 1923

3 Sheets-Sheet 3

Fig. 12.



Fig. 11.



Fig. 10.



Fig. 13.



Fig. 14.



INVENTOR  
PAUL LÉON HULIN  
BY

*Léon, Kellner & Mothé*

ATTORNEYS

## UNITED STATES PATENT OFFICE.

PAUL LÉON HULIN, OF GRENOBLE, FRANCE.

## PREPARATION OF SODIUM.

Application filed November 26, 1923, Serial No. 676,887, and in France December 16, 1922.

This invention relates to improvements in electrolytic processes for the preparation of sodium in which this metal is formed in the liquid condition on a cathode made of solid metal from which it becomes detached under the form of molten globules.

Its main application is the production of sodium by electrolysis of a bath of caustic soda (NaOH) in fusion.

10 The invention may also be applied to the electrolysis of any sodium compounds in molten condition such as the carbonate, chloride, etc., whether they are separately treated or mixed together or whether other suitable materials are added to the same.

In the case of the electrolysis of soda, as noted by Castner, the production of sodium rapidly diminishes when the temperature of the bath of electrolysis rises; it is therefore necessary that this bath should not be heated much above the melting point of soda if it is desired to obtain the best possible output.

25 The heating produced by the Joule effect is sufficiently regular and adjustable. It is easy to devise the apparatus in such a manner that it suitably dissipates any excess of heat.

But even if the temperature has been maintained below the proper limit, the production of sodium may diminish owing to irregularities or trouble in the operation of the apparatus; this would cause an abnormal rise of temperature and two prejudicial conditions then arise which aggravate each other and which conjointly act to further reduce the output.

The decrease of the production is thus, sometimes, rapid and considerable.

40 I have discovered that the main cause of this special trouble is due to the fact that the sodium, formed at this moment, no longer forms a layer adhering on the cathode, but on the contrary becomes detached from the latter, being divided into fine particles scattered throughout the bath where it immediately reacts on OH thus forming hydroxide (NaOH) and at the same time giving off a great amount of heat.

50 This phenomenon exists in all apparatus which electrolyze soda in a continuous manner. Its frequency is very variable; it depends on the foreign bodies contained in the electrolyte, on the particular arrange-

ments of the apparatus, on the method of 55 operation, etc.

For remedying this difficulty, various means have been proposed: Stoppages, with or without special cooling, until return to the normal temperature, this being only a 60 momentary remedy. Renewal of the electrolyte with complete cleaning of the apparatus, this being costly and laborious. Replacement of the cathode or periodical pickling of the latter by immersion in water 65 where it resumes its metallic aspect and, with it, its property of giving out again sodium with a suitable efficiency.

This latter process, forming the subject matter of a previous patent of mine is still 70 considered valuable and is in current use.

Although constituting an important improvement, said patented process is not easily applicable to apparatus of the Castner type; moreover, in apparatus of large dimensions, the operations for removing, pickling and inserting the cathodes require 75 somewhat laborious and delicate work, which may cause injury to the cathodes manipulated, losses in soda, etc.

80 The process and devices forming the subject-matter of my present invention are adapted to remedy all these drawbacks. By this invention, I may, without removing the cathode, reestablish the formation of sodium in the form of an adherent layer or of globules sufficiently massive for resisting the action of the bath tending to detach the sodium from the cathode. I thus obtain an output in sodium higher than by any of the 85 previous processes, as well as a reduction in the consumption of soda.

90 The new process consists, substantially, in periodically operating a superficial oxidation of the cathode by causing such cathode to act as an anode during a limited time, using for this purpose a very reduced amount of electricity relatively to the amount employed for the electrolysis.

95 This process can be carried out by means of three main methods of operation.

100 1. By reversing the direction of all the current between the anode made of iron (or of nickel or very slightly oxidizable alloy) and the copper cathode, during a very short time, say between two and ten seconds.

105 2. By reversing the direction of the current between the anode and cathode on a

portion only of the electrolyzing current, the other portion being branched from the electrolysis circuit and the duration of the reversal can be increased in proportion to this branching.

3. By momentarily forming special connections comprising one or more twin electrodes and one or more auxiliary electrodes.

The two first methods of operation can be 10 carried out by means of any known or suitable devices.

The third method of operation is carried out by momentarily connecting the cathode with the anode and by causing these two 15 electrodes thus electrically connected to act as a single anode, or as twin anodes, relatively to another suitable electrode functioning, at that moment, as a cathode common to such anodes. This cathode, which performs its special function intermittently, 20 will be designated hereafter under the name of auxiliary cathode.

After having maintained the cathode in electric connection with the anode during a 25 certain time, this cathode and this anode are caused to resume their independence and their normal function.

It is possible to operate the individual 30 cells or units of such an apparatus one by one without affecting the others and without sensibly modifying the intensity of the current of the general supply circuit in which the direction of the current can thus remain constant.

35 As will be seen hereafter, the invention will improve the operation and efficiency of all the types of apparatus producing sodium by electrolysis.

For applying this process, the apparatus 40 is furnished with a system of connections and movable contacts, specially combined, by the operation of which the electrodes are periodically connected according to the principle which has just been described.

45 The accompanying drawing illustrates, by way of example, the application on well-known types of apparatus, of the principles and essential arrangements of the distribution of the current alternately on two 50 cathodes, with the cathode-anode connection, in accordance with the present invention.

In said drawings, Figs. 1, 2 and 3 are vertical sections through an electrolytic cell for carrying out my present invention, 55 these three figures differing only as to the electrical connections; Figs. 4 and 6 show another form of such cell with connections corresponding to those of Figs. 1 and 3 respectively; Fig. 5 illustrates the third arrangement of electrical connections for the cell shown in Figs. 4 and 6; Figs. 7, 8 and 9 are views corresponding to Figs. 4, 5, and 6 respectively, illustrating the use of my invention with cells of the Castner type; Figs. 60 65 10, 11 and 12 are views corresponding to

Figs. 4, 5, and 6, illustrating still another form of electrolytic cell and the different electrical connections employed therefor; and Figs. 13 and 14 are views corresponding to Figs. 4 and 6, showing a further suitable 70 form of electrolytic cell.

Each of the electrolytic cells illustrated comprises essentially a vat A containing the caustic soda in fusion, an anode B made of iron or nickel or a very slightly oxidizable 75 alloy, on which oxygen evolves, a cathode C preferably of copper (or a copper alloy) on which are formed at the same time the sodium (liquid) and the hydrogen (gaseous), and a header, receiver or bell D, in which is 80 collected the sodium given off.

The standard Castner apparatus, Figs. 7 and 9, comprises moreover a wire gauze diaphragm F interposed between the electrodes for separating the oxygen from the sodium and hydrogen which ascend close around the cathode.

Figs. 10 and 11 illustrate another apparatus having an immersed cathode provided with such a diaphragm or separator F suspended from the collecting ring D.

With each of these apparatuses is associated a combination of fixed contact pieces b, c, l, e and of movable contacts h, j, k, the whole forming a switching system of 90 peculiar novel operation.

These contact pieces and contacts may moreover be arranged in a manner other than that shown and they can be spaced apart instead of being arranged in groups.

For these connections and these movable contacts any suitable detail arrangements can be adopted, the contacts can be constituted by bars, blades, pins, handles, etc., and use can be made of all the necessary operating accessories which may, if desired, be independent of each other, common to or rigid with each other and even automatic.

The auxiliary cathode is composed of a metallic member immersed in the electrolyte as would be a working electrode.

By way of example, such an auxiliary cathode is shown at E in Figs. 1, 2 and 3.

It is arranged about the anode, but it might occupy other positions. This auxiliary cathode is constituted, here, by a sheet iron ring provided with a current supply conductor i which is connected at its outer end to a terminal or contact piece e by which the current is supplied or is interrupted at will.

The working current is supplied to the anode B directly through a conductor a, without necessity of interposing any switch in the circuit. A branch circuit for this working current is established at f and leads to the contact piece b.

When the working cathode C is in a period of production, the contacts occupy the position shown in Fig. 1; the current which

passes from the anode to this cathode within the bath, issues through *g* and comes to the contact piece *c* connected at this moment to the main *d* by the movable contact *h*.

Figs. 1, 4, 7, 10 thus each represent an apparatus in a condition of normal production owing to the position of its switching system.

When the output in metal seems to diminish, or when the temperature of the bath tends to rise, or for the purpose of avoiding these objectionable occurrences, normal working is re-established or ensured by operating as follows:

The auxiliary cathode *E* is caused to become active by first connecting through the movable contact *j*, the contact piece *e* to the contact piece *l*, position of Fig. 2. The current then branches in the bath by passing, on the one hand, from the anode *B* to the cathode *C* and, on the other hand, from the same anode *B* to the auxiliary cathode *E*. This position, however, is only a transitory position adapted to avoid the interruption of the main supply current. It is the position illustrated in Figs. 2, 5, 8 and 11.

The movable contact *h* is then removed and *b* is connected to *c* by means of the contact *k*, position illustrated in Figs. 3, 6 and 9; the work cathode *C* is then connected with the anode *B* by *g*, *o*, *b*, *f*. The apparatus comprises therefore at this moment two twin anodes emitting together the main current in the mass of the bath towards the auxiliary cathode.

The cathodic-anodic substitution connection allows to obtain on the spot, in the most practical manner, the superficial oxidation of the working cathode giving the high output which results from this oxidation.

The duration of the oxidizing connection varies with the arrangement of the apparatus, the relative position of the electrodes in action and their dimensions, the intensities of current which pass through them, the condition of the electrolyte, etc.

One minute will usually be sufficient for each oxidizing operation with an average of six sodium producing operations in twenty-four hours; but it is preferable, in each plant to determine and to regulate at the beginning, by trials, the duration and frequency which are suitable for given apparatuses and electrolytes.

The oxidation of the cathode is caused to cease and the apparatus to restart its normal operation, by effecting in reverse direction the switching movements described above. For this purpose the contact bar *h* is first removed and the bar *h* is replaced on the contact pieces *c* and *l*, so as to thus pass again through the transitory position of Fig. 2. The contact piece *j* is subsequently removed, thus restoring the apparatus to the position shown in Fig. 1.

According to the present process, the oxidation of the cathode must be effected carefully in order to remain superficial and without notably corroding this electrode.

This condition is already ensured by the principle of the process itself, but it is usefully completed by suitable arrangements the two principal ones of which are:

1. The position of the auxiliary cathode outside the anode, this having for its effect to cause the main mass of the current to pass directly from the anode *B* to the auxiliary cathode *E* so much the more as the intensity of the current which passes from the electrode *C* to the auxiliary cathode *E* is, moreover, reduced owing to the position of *C* within *B*.

The oxidation of the cathode *C* thus remains superficial and uninjurious if care is taken to suitably limit, on the other hand, the duration of this oxidation.

2. The insertion between the contact piece *b* and the anode *B* (that is to say on the line *f*) of a resistance, which can be adjustable, through which is limited at will the intensity of the current passing through the cathode *C* during the operation of oxidation of the latter. It has not been considered necessary to specially illustrate this resistance.

By means of this regulating device it is possible to reduce at will the rapidity of oxidation of the cathode; this oxidation is thus rendered more regular and prejudicial corrosion is easily avoided.

These various means can be employed separately or combined.

An interesting form of carrying out the invention consists in applying certain parts of the apparatuses themselves to the intermittent function of auxiliary cathode.

The vat *A* (Figs. 4 and 6) is preferably used as auxiliary cathode, this usually rendering unnecessary the special electrode *E*.

For that purpose, the vat *A* (Figs. 4, 7 and 10) is connected to the terminal or contact piece *e* by a conductor *i* of sufficient cross section, and the most simple and most suitable auxiliary cathode is thus obtained.

This modification is applicable to most of the apparatus in use in the industry.

The switching operation is effected as previously described.

The connections of Fig. 4 are changed to those of Fig. 6, and vice versa, preferably through an intermediate transitory position, Fig. 5, in order to avoid the serious inconveniences of an interruption of the main current, this might moreover be obtained by another momentary connection effected at another place.

It is also possible to use as auxiliary cathode, separately, or preferably combined with the vat, other members such as the sodium

receiver D and especially the wire gauze diaphragm F when this separator is used between the anode B and the cathode C, as in the standard Castner apparatus (Figs. 7 and 9) or in any other apparatus, for instance that illustrated in Figs. 10 and 12.

Figs. 7 to 12 illustrate, in the working and oxidizing positions, the apparatus to which are applied the combinations corresponding to these modifications of the invention.

The vat A is caused to act as main auxiliary cathode, by connecting it to the branch *d* of the circuit, as already described, by a contact bar *j* connecting the contact piece *e* to the contact piece *l*.

Moreover, there is provided a contact piece such as *m* and a conductor *n* forming a fixed or variable resistance, connected to the header or receiver D and, by the latter to the wire gauze diaphragm F, which is suspended therefrom.

For effecting the oxidation of the main or working cathode C, by means of these combined auxiliary cathodes (compound auxiliary cathode), the vat A is connected, as already explained, to the contact piece *l* by the movable contact *j* inserted between the contact pieces *e*, *l* (Figs. 8 and 11); the conductor *n* is connected to *e* and A by means of a suitable contact such as *o* or any other equivalent contact inserted between *m* and *e* (Fig. 9) or *m* and *l* (Fig. 12), after which the blade *h* is removed and the contact *e* is placed in position. The connections shown in Figs. 9 and 12 are thus obtained.

The current then takes several paths through the bath. The main portion passes from B to E; a fraction passes from B to F and to D. The small fraction of the current which effects the cathodic oxidation and is controlled at will by the resistance *n*, passes from C to F and from C to D and to A.

The return to the working phase is effected as previously described by bringing back the connections to the positions of Figs. 7 and 10.

The function of auxiliary cathode is carried out in a still simpler manner when the apparatus comprises a system of multiple electrodes operating parallel in group in the same vat.

In this case, for producing the momentary oxidation of one of the cathodes, use can be made as auxiliary cathode of one of the other cathodes in action, or a group of other cathodes, which will thus work with overload during this time.

This modification is illustrated, by way of example, in section and in elevation in Figs. 13 and 14. These drawings will be sufficient for allowing the arrangements and operation to be understood.

The anode is composed of several assembled parallel elements B—B—B—B, which

receive through *a* the current of the main circuit.

In the intervals are arranged the cathodes C<sup>1</sup>, C<sup>2</sup>, C<sup>3</sup>. In the position shown in Fig. 13, which is that of normal working, these cathodes are connected by the contact pieces *c*, movable contacts *h* and contact pieces *l*, to the conductor *d*.

For effecting the oxidation of one of the cathodes, the cathodes C<sup>1</sup> for instance (first of the group), the movable contact *h* is placed in the position *k*, Fig. 14, this establishing a connection of this cathode with the conductor *a*. The cathode C<sup>1</sup> then acts as anode at the same time as the anodes B, thus constituting a partial element of the anodic electrode, and it is these latter anodes B which give passage to the main mass of the current, all according to the principle of the invention.

During this time, the other cathodes C<sup>2</sup> and C<sup>3</sup> operate together as auxiliary cathode by receiving all the current.

When the cathode to be oxidized has been subjected to this treatment, it is replaced in productive service condition by the reverse operation which consists of replacing at *h* the movable contact *l*, this bringing back the apparatus to the position of Fig. 13 which corresponds to normal operation.

The other cathodes are successively treated in the same manner.

Of course this modification does not exclude the possibility of causing any other auxiliary cathode to participate at the same time in the operation, particularly the vat of the apparatus which contains the groups of electrodes.

The principles and means described are of course applicable to all types of apparatus comprising, in any number, multiple electrodes or electrodes composed of assembled elements which can be separated or connected in various ways for effecting the operations in separate units, in fractions, or in groups, according to numerous modifications which can be realized in the carrying out of the invention.

Moreover, it is possible to insert or use in conjunction with the means described any other means, parts or accessories without changing the principle of the said invention. Besides, the shapes of the apparatus, details, dimensions and certain materials used may be varied according to circumstances and applications.

#### Claims—

1. In the production of sodium by the electrolysis of a bath of molten caustic soda with the use of a copper cathode and a slightly oxidizable anode, the step which consists in effecting periodically, with the electrolytic bath itself, a superficial oxidation of the cathode.

2. In the production of sodium by the

electrolysis of a bath of molten caustic soda with the use of an oxidizable cathode, the step which consists in periodically effecting, in the electrolyzing bath, on said cathode, 5 an anodic reaction by the momentary action in the suitable direction of an amount of electricity limited to the formation of a layer of superficial oxide.

3. In the production of sodium by the electrolysis of a bath of molten caustic soda with the use of a copper cathode and a slightly oxidizable anode, the step which consists in periodically reversing the direction of the electrolyzing current between 10 said anode and said cathode, the current flowing during such reversal being limited to about that necessary for the superficial oxidation of copper.

4. In the production of sodium by the electrolysis of a bath of molten soda, the step which consists in periodically effecting on the cathode, in the electrolyzing bath, a superficial anodic reaction by the momentary action in the suitable direction of a current 25 the intensity of which is materially smaller than that of the electrolyzing current.

5. In the production of sodium by the electrolysis of a bath of molten soda, the step which consists in periodically causing 30 the cathode to act as anode, during a limited time under a suitably directed portion of the electrolyzing current, the other portion of this current being deflected and passing outside the cathode treated.

35 6. In an electrolytic process performed with the aid of an anode, a main cathode, and an auxiliary cathode, the step which consists in periodically connecting both the anode and the main cathode with the positive pole of the source of electricity while the auxiliary cathode is connected with the negative pole, to effect during that time a reversal of the current at the main cathode.

7. In an electrolytic process performed 45 with the aid of an anode, a main cathode, and an auxiliary cathode, the step which consists in periodically connecting the anode with the main cathode through a resistance, the cathode thus becoming temporarily an anode when the auxiliary cathode is connected with the negative pole of the source of electricity.

8. In an electrolytic process performed 55 with the aid of a main cathode, an auxiliary cathode, and a third electrode placed between said main and auxiliary cathodes, the operation which consists in normally connecting the negative pole of the source of electricity with said main cathode and periodically connecting the latter with the

positive pole while the negative pole is connected with the auxiliary cathode to produce a temporary flow of current in the opposite direction at the main cathode.

9. In the production of sodium by the 65 electrolysis of a bath of molten caustic soda, with the use of a copper cathode and a slightly oxidizable anode, the step which consists in periodically connecting one of those conducting elements of the apparatus 70 which are in contact with the bath, with the negative pole of the source of electricity while said cathode is connected temporarily with the positive pole.

10. In electrolytic processes for the 75 preparation of sodium by the electrolysis of a bath of molten caustic soda, with an electrode consisting of a plurality of units, normally functioning as cathodes, and a slightly oxidizable anode, the step which consists 80 in temporarily and successively causing said units to assume anodic functions to produce the superficial oxidation thereof.

11. In electrolytic processes for the preparation of sodium, by the electrolysis of a bath 85 of molten caustic soda, with a cathode consisting of a plurality of separate electrodes, and a slightly oxidizable anode, the step which consists in temporarily and successively distributing the cathodic charge 90 among certain of said electrodes while the remaining ones are caused to function as anodes to produce the superficial oxidation thereof.

12. In electrolytic processes employing an 95 anode, a main cathode, and an auxiliary cathode which is inactive during the normal electrolytic operation, the step which consists in periodically connecting the anode with the main cathode so that the latter temporarily assumes anodic functions while at 100 the same time connecting the auxiliary cathode with the negative pole of the source of electricity.

13. In electrolytic processes employing an 105 anode and a cathode composed of a plurality of units having independent connections normally leading to the negative pole of the source of electricity, the step which consists in temporarily disconnecting successively a 110 part of said units, from such negative pole, and connecting them with the anode, while the other units continue to function as a cathode.

The foregoing specification of my "im- 115 provements in the preparation of sodium" signed by me this 14th day of November, 1923.

PAUL LÉON HULIN.